

April 11, 1944.

F. C. HENDERSON

2,346,579

## CERAMIC PROCESSES

Filed April 10, 1942

FIG. I.



FIG. 2. 5 7



### WATER REPELLENT AREA

## WATER GLAZE

WATERPROOF GLAZE  
WATER REPELLANT AREA

INVENTOR.

FREDERICK C. HENDERSON

BY

WATERGLAZE FIG. 3.

BY  
Chas K. Davies & Son  
Attns.

## UNITED STATES PATENT OFFICE

2,346,579

## CERAMIC PROCESS

Frederick C. Henderson, East Liverpool, Ohio,  
assignor to The Hall China Company, East  
Liverpool, Ohio, a corporation

Application April 10, 1942, Serial No. 438,473

8 Claims. (Cl. 117—40)

My present invention relates to an improved Ceramic process or method of decorating or ornamenting chinaware and similar articles. The process or method involves the application of two or more coats of ceramic glazes, one on each of adjoining areas of the surface of the article to be decorated, and before the glaze on the cast or molded article is fired.

These glazes are applied to the surface of the ware in such manner that the adjoining edges of adjacent, and possibly contrasting glazed areas, lines, figures, etc., will not merge or run together during the subsequent firing of the decorated article; but on the other hand, the procedure according to my process insures clear cut meeting or contacting lines and distinct lines of demarcation between adjoining edges of the two glazed areas, thus providing the required decorations or ornamentations with neat and artistic finishes.

The adjoining glazed areas, lines, figures, etc., applied to the surface of the ceramic ware, are usually of different natures and characteristics, and made up in contrasting colors; or in other instances the two or more adjoining glazes applied to the ware may be of different shades of the same color. For instance, and as a simple illustration of my invention, I have shown in the accompanying drawing a ceramic bowl, which may have an interior glaze of one color, an exterior glaze of another color, and the rim or top edge of the bowl is to be decorated with another glaze of another color.

In order to facilitate understanding of the invention and as one illustration of the manner in which the steps in the process or method of my invention are carried out, I first employ and apply to a specific area of the surface of the unfired ware to be decorated or ornamented a ceramic glaze that is waterproof, and the ingredients of the glaze are carried in a vehicle that is water-repellent when applied to the article for decorative purposes. An adjoining area on the surface of the article to be decorated is next coated with a ceramic water-glaze. After the two (or more), glazes have thus been applied to the bowl, the latter is fired and the finished article is found to have clear and clean cut lines of contact between adjoining glazed surfaces of the bowl. Thus in the process of decorating or ornamenting the porous unfired ware a minimum of two successive steps are employed, the first involving the application of a glaze including a water repellent mobile liquid vehicle which penetrates the porous surface of

the ware; and the second step involves the application of a glaze having a penetrating vehicle that is incapable of mixing or merging with and is repelled by the vehicle of the first glaze. As an illustration of two immiscible vehicles that may be employed in the steps of my process the first vehicle may be liquid paraffin wax, and the second vehicle may be water; but it will be understood that I do not limit my invention to these specific vehicles.

In the accompanying drawing I have illustrated one mode that may be employed in applying the water-proof and water-repellent glaze to the porous ceramic ware or unfired china bowl, but it will be understood that other means may be employed if they are suitable for my purpose.

Figure 1 is a sectional view of a tank containing the water-proof and water-repellent glaze, 20 showing an elevated screen-table on which the circular rim or top edge of the bowl is "touched" to absorb by capillary attraction the glaze.

Figure 2 is a top plan view of the tank in Figure 1, showing by circular dotted lines the relative 25 position of the rim or edge of the bowl.

Figure 3 is a diagrammatic, exaggerated, view illustrating the water-repellent area between a waterproof glaze and two water-glazes.

The waterproof glaze is made up of, or prepared principally from a dry powder glaze which is incorporated in and carried by a vehicle in the nature of and having the characteristics of melted wax, the glaze mixture being a mobile liquid approximating the thickness or viscosity of thick oil. I find that paraffin is a preferred vehicle or carrier for the ceramic glaze ingredients, because it not only is waterproof and a water-repellent, but it also is capable of resisting the action of acids and alkalis that might be used in the ceramic art.

This dry powdered glaze material that is incorporated in and employed jointly with the melted paraffin wax may include flint, feldspar, whiting, clay and magnesite, or other suitable glaze or enamel ingredient, without a colorant or with a colorant.

These glaze materials are first ground very fine in water, then dried out in suitable manner, and finally ground or crushed to a very fine powder.

To prevent these materials, as fine powders, of the glaze from coalescing or adhering, or forming lumps, while in suspension in the glaze mixture, I utilize a deflocculent in the glaze mixture, such as zinc naphthenate, to maintain a

uniform consistency throughout the liquid glaze mixture, which insures a smooth glaze surface when applied to the ware to be decorated, when the ware, as a bowl, is fired.

To counteract the odor arising from the zinc naphthenate in the mixture I may add a deodorant or counterodorant to the mixture, such as distilled pine oil which is satisfactory for the purpose.

I have attained very satisfactory results in a ceramic glaze employing the ingredients of the mixture in approximately the following quantities:

|                                                                                                     | Per cent |
|-----------------------------------------------------------------------------------------------------|----------|
| Paraffin                                                                                            | 50       |
| Dry powdered glaze                                                                                  | 50       |
| Zinc naphthenate                                                                                    | 2        |
| Pine oil in the ratio of 2½ cubic centimeters to 1000 grams of paraffin, and a colorant if desired. |          |

In one mode of preparing this ceramic glaze the desired quantity of paraffin in the form of wax is melted in the tank 1 by use of the electric heaters 2 located beneath the central well of the tank, and as soon as the paraffin has been melted and liquified to the desired consistency, the dry powdered glaze, the deflocculent, and the deodorizer, as well as a colorant, are added gradually to the liquid paraffin. By means of a rotary agitator 3 that is operated by an electric motor 4 clamped on an edge of the tank the various ingredients are stirred and agitated and suspended in the liquid paraffin, it being understood that the heaters 2 are utilized to maintain the liquid consistency of the paraffin, not only while the wax-glaze is being mixed, but also while the glaze is being applied, if necessary.

While heating, the liquified mixture is stirred or agitated until the various ingredients or constituents are uniformly distributed in a homogeneous, smooth, fluent compact mass, especially in the upper portion of the tank above the agitator or rotary impeller 3. To aid in preparing this fluent texture of the waterproof glaze and in enhancing the uniformity in consistency throughout the glaze mixture, a horizontal screen-table 5 may be vertically reciprocated by means of the cam devices 6, 6, which support the screen-table. These cam devices may be actuated manually, automatically, or by treadles, or the screen-table may be elevated and lowered in any other suitable manner. The screen-table, which is reticulated, may be of muslin, copper or fine bronze screen material of approximately eighty mesh, and the horizontally supported screen may be vertically reciprocated, as a separator or strainer, in the upper bulk portion of the wax glaze, above the impeller or agitator, to assist in maintaining the solids of the glaze in suspension and assist the deflocculent in preventing the grains or dust of different powdered materials of the glaze from coalescing or adhering one with another. After the waterproof glaze has been liquified to a consistency or viscosity of thick oil, the solids of the glaze remain in suspension and a minimum of stirring or agitation is required to maintain the glaze mixture in working condition. While the heaters 2 maintain the desired thickness of the paraffin carrier or vehicle and the solids are suspended in compact uniform homogeneous mass, the waterproof glaze is applied to the ceramic article.

In the drawing I have for convenience of illustration shown a chinaware bowl B having a circular rim R, to which rim or edge of the bowl the waterproof glaze is to be applied. First 5 the cams 6, 6, are employed to lift the submerged dotted-line screen to the full-line elevated position in Figure 1, in order that the flat horizontal screen with its covering or coating of mobile and fluent waterproof liquid glaze, 10 may be used as a "dipping" table for the bowl. The bowl in inverted position is then "touched" or lightly dipped, by hand, in contact with the liquid glaze that is supported on the top of the screen table, and then the bowl is removed. By 15 capillary attraction of the liquid portion of the glaze, wax is absorbed by the rim R of the bowl B, and the solids of the glaze are applied to the rim or edge R to provide the coating. In Figure 3 this waterproof glaze is indicated, and at the 20 sides of this glaze two hair-lines are shown to indicate water-repellant areas, which areas are formed by the liquid content of the waterproof glaze which "creeps" slightly, out, beyond the solid body of the glaze that is made up of the 25 different powdered materials heretofore enumerated. The liquid content or vehicle of the glaze contacting with the bowl penetrates the surface of the porous ware, and this "creeping" 30 of a portion of the liquid content provides a thin film that forms the water-repellant area or hair line. This contact line caused by creepage of the vehicle is sufficient to repel a second glaze and thereby eliminate possibility of merging the first and second glazes during subsequent 35 firing of the bowl.

In Figure 3, in addition to the waterproof glaze with its two water repellent areas, I also indicate two water glazes, one at each side of the waterproof glaze. These water glazes may 40 contain the same ingredients as are included in the waterproof glaze, but they are carried in water as a vehicle; or these water glazes may be standard types of glazes, and like the waterproof glaze, they may also be colored, or non-colored. In either event, because of the water 45 content of the water glaze, when the upright bowl B is dipped in a water glaze to receive an exterior glaze, for instance, the moisture of the water glaze is stopped and repelled when it contacts with the hairline of paraffin that forms the water repellent area indicated in the drawing.

The applied glazes of course solidify by cooling or drying so that the ware with the glazes 55 applied is ready for the usual firing of the bowl to insure the smooth fired finish of the glaze in the ornamental or decorative features of the bowl.

In this manner the ware, as a china bowl, may be decorated or ornamented by the application of glazes in lines, figures, bands, etc., either in contrasting colors, in differing shades of the same color, or the glazes may be colorless, and 60 they are applied to a variety of metallic or non-metallic ceramic articles.

While I have confined my description to the use of an organic vehicle as molten or melted paraffin wax as the carrier for the ingredients 65 forming the inorganic glaze, it will be understood that other suitable materials may be employed. Further, while I have referred to zinc naphthenate as the deflocculent employed to reduce the tendency of the inorganic portion of 70 the waterproof glaze mixture to separate from

the organic carrier or vehicle, other suitable deflocculents, such as linseed oil may be introduced to and incorporated in the mobile liquid glaze.

The mixing and dipping tank and the conventional accessories associated therewith in the exemplifying drawing are merely for illustrative purposes, and it will be understood that I do not confine myself to the use of such illustrated equipment.

Having thus fully described my invention, what I claim as new and desire to secure by Letters Patent is:

1. The steps in the process of decorating unfired porous ware which consist in successively applying to adjoining surface-areas mobile liquid glazes which include two immiscible vehicles at least one of which penetrates the ware and forms an intermediate non-glazed area to prevent merging of the glazes during firing; drying the applied glazes; and finally firing the glazed ware.

2. The steps in the process of decorating unfired porous ware which consist in applying to a surface-area a glaze including a mobile liquid vehicle which penetrates the ware, creeps beyond the glaze, and thereby forms a non-glazed edge at the border of the glaze; then applying to an adjoining surface-area a glaze having a liquid vehicle that is incapable of mixing with the first vehicle and finally firing the glazed ware.

3. The steps in the process of decorating unfired porous ware which consist in applying to a surface-area a glaze including a waterproof mobile wax as a vehicle which penetrates the ware, creeps beyond the glaze and thereby forms a water-repellant non-glazed edge at the border of the glaze; then applying to an adjoining surface-area a glaze having a water-vehicle; drying the applied glazes; and finally firing the glazed ware.

4. The process of decorating unfired ceramic ware and similar porous articles which consists in applying to the article a penetrating waterproof glaze which creeps to form a coating having a water-repellant non-glazed edge, applying a penetrating water-glaze to a surface area adjoining said edge and thus forming an intermediate non-glazed area to prevent merging of the two glazes during firing; and finally firing the article.

5. The process of decorating porous unfired ceramic ware which consists in applying a penetrating waterproof glaze of one color which creeps and forms a coating having a water-repellant non-glazed edge; then applying a penetrating water-glaze of another color to a surface-area adjoining said edge and thus forming an intermediate non-glazed area to prevent merging of the two glazes during firing; and finally firing the ware.

10 6. The process of decorating unfired porous ware which consists in heating and agitating a mobile liquid waterproof glaze in a container; applying this glaze to the ware to penetrate its surface and form a coating having a non-glazed water-repellant edge; heating and agitating a water-glaze in a container, applying the water-glaze to a surface-area adjoining said edge and thus forming an intermediate non-glazed area to prevent merging of the two glazes during firing; and finally firing the glazed ware.

15 7. The process of applying glazes of various colors on adjoining surface-areas of unfired porous ware which consists in dipping a surface-area of the ware into a mobile liquid glaze of one color and including a water-repellant vehicle which penetrates the ware and creeps beyond the glaze thereby forming a non-glazed waterproof line beyond the solid portion of the glaze; then applying a glaze of another color and having a water vehicle to an adjoining surface-area of the ware whereby the second vehicle is repelled at said line to prevent merging of the glazes; drying the glazes; and finally firing the glazed ware.

20 8. The process of decorating unfired porous ceramic ware which consists in heating a glaze mixture including a waterproof vehicle in a container, dipping a surface-area of the ware in said mixture whereby the vehicle penetrates the ware and creeps beyond the glaze of the mixture to form a water-repellant non-glazed line beyond the solid portion of the glaze, then applying a glaze of another color and having a water vehicle to an adjoining surface-area of the ware whereby the second vehicle is repelled at said line to prevent merging of the glazes, drying the glazes, and finally firing the glazed ware.

FREDERICK C. HENDERSON.